

1

2,773,035

## SOLUBLE OIL COMPOSITIONS

Stanley P. Waugh, Westfield, N. J., assignor to Tidewater Oil Company, a corporation of Delaware

No Drawing. Application December 12, 1951,  
Serial No. 261,381

11 Claims. (Cl. 252—33.3)

The present invention relates to improved soluble oil compositions.

In the metal fabricating, cutting and related arts, use is made of emulsions which function to lubricate and cool the metal and cutting tools used in turning, drilling, grinding and similar operations. In many of such operations, the emulsions are prepared by emulsifying a suitable soluble oil with a relatively large proportionate amount of water. The soluble oils employed usually contain as essential ingredients a lubricating base, an emulsifying agent and water, said ingredients being generally employed in rather well defined proportionate amounts so that the soluble oil itself will be a homogeneous solution stable against ingredient separation and will readily emulsify with formation of a stable emulsion when added to and agitated with a relatively large proportionate amount of water. Although the art is aware of soluble oils that contain, as the lubricating base, materials other than of petroleum origin, the most widely used, to my knowledge, are soluble oils in which the lubricating base is of petroleum origin and may comprise a mineral oil of the lubricating oil boiling range, a spindle oil, a pale oil or types similar thereto. Lubricating bases used for soluble oils include distillate oils, derived from petroleum crudes, that vary over a rather wide range of viscosity, the particular viscosity employed being determined primarily by the contemplated usage of the soluble oil. For most purposes, however, lubricating bases having viscosities not exceeding about 500 SUS at 100° F. have been employed, illustrative examples thereof being distillate oils having a viscosity of about 100 SUS at 100° F., and one reason for preferred usage of such mineral oils of the lower viscosity characteristics is that, in general, they may be rendered emulsifiable more readily than higher viscosity oils.

The art is also aware of many emulsifying agents usable in soluble oils to facilitate the dispersibility and emulsifiability of the lubricating base with water. In illustration, emulsifying agents used for soluble oils include metal or onium base soaps such as the alkali metal or onium base naphthenates and sulfonates. As examples of the organic soaps, the oleates of alkylol amines such as the di- and tri-ethanol amine oleates have been employed and, of the metal soaps, wide use has and is still being made of water-soluble alkali metal soaps of organic acids such as the fatty acids, sulfonic acids, naphthenic acids and the like, with sodium and potassium soaps of such acids being more specific illustrations.

In addition to soluble oils that consist of a lubricating base, an emulsifying agent and water, the art is aware of soluble oils that contain additional ingredients to impart certain desired properties or characteristics. Thus, numerous soluble oils, and particularly those containing a metal soap as an emulsifier, contain coupling agents adapted to facilitate dispersion of the emulsifying agent in the oil whereby the resultant soluble oil is a homogeneous product stable against ingredient separation. Coupling agents used include alcohols of the aliphatic type, such as the propanols and butanols, polyhydric alco-

2

hols such as the glycols and, more specifically, diethylene glycol, and glycol ethers such as diethylene glycol monobutylether. Such coupling agents have been used singly or in combination and illustrative of use of such agents in combination is diethylene glycol with diethylene glycol monobutyl ether. Especially suitable results are obtained by use of such a combination in soluble oils in an amount of about 0.3 to about 3 percent of the polyhydric alcohol and an amount of the alcohol ether of from about one to about five times that of the polyhydric alcohol.

Water, in addition to being an essential ingredient in soluble oils as afore-discussed, must be correlated with the remaining ingredients of the composition in order to provide a soluble oil that is homogeneous and stable against ingredient separation and which readily forms stable emulsions when added to relatively large proportionate amounts of water to form the composition ready for use in cutting operations and the like. For example, soluble oils that contain water, but in an insufficient amount, have a tendency to gel, whereas soluble oils that contain an excessive amount of water usually evidence instability caused by the soap separating out of solution. Thus, and with respect to a particular soluble oil composition, a rather well defined range of water will be tolerated thereby. Addition of water to the composition in an amount in excess of that tolerated leads to formation of a cloudy or hazy appearance and oftentimes stratification occurs due to ingredient separation. Generally speaking, the more water, within limits, which can be tolerated by a soluble oil in stable solution the more stable will be the emulsion resulting from later addition of the soluble oil to a relatively large proportionate amount of water necessary to prepare it for use. In certain soluble oil compositions increased amounts of water can be tolerated thereby by increasing the soap content but use of such an expedient is not desirable from an economic viewpoint as soap is one of the more expensive of the ingredients used in soluble oils. Provision of soluble oils having increased tolerances for water without necessitating use of increased soap content are desirable not only from an economic viewpoint but also because they minimize the need for critical control during manufacture as compared to preparation of soluble oils having narrower ranges of water tolerance.

It is an object of the present invention to provide novel, stable homogeneous soluble oil compositions that readily form stable emulsions with a relatively large proportionate amount of water, and which compositions possess an exceedingly wide range of water tolerance.

Another object is to provide such soluble oil compositions that, in addition to having an exceedingly wide range of water tolerance, possess a relatively high load carrying capacity.

Still another object is to provide stable, homogeneous soluble oil compositions that contain a novel combination of ingredients whereby the compositions possess an exceedingly wide water tolerance and readily form stable emulsions that possess an unexpectedly high load carrying capacity.

The present invention relates to compositions, adapted for use as soluble oils, that possess desired properties as afore-discussed and which result by use as a lubricating base in the compositions of a suitable solvent extract of petroleum origin. As described more fully hereinafter, the lubricating base employed may consist of the solvent extract or, more preferably, a liquid mixture of the extract and a mineral oil. Hence, the compositions embodied herein comprise a lubricating base, an emulsifying agent, water in an amount sufficient to inhibit the composition against gelation but less than an amount sufficient to induce ingredient separation, and are further characterized in that the lubricating base contains a solvent extract of petroleum origin.

Mineral oil solvent extraction processes are well known to those experienced in the art and since the extraction processes per se are not a part of the present invention it is not deemed essential to describe such processes in detail herein. For purposes of illustration, however, such solvent extraction processes entail use of solvents such as beta, beta-di-chloroethyl ether, furfural, phenol and other suitable solvents under extraction conditions to preferentially extract from the mineral oils the aromatic-containing molecules therein. In more specific illustration, furfural is a widely used and typical extraction solvent and, hence, for purposes of illustration, extracts derived from mineral oils by use of such a solvent are employed herein to describe this invention.

The improved soluble oil compositions obtained by practice of the present invention are illustrated by the data in the following tabulation which includes compositions as embodied herein as compared to a conventional soluble oil in which the lubricating base component was devoid of a solvent extract of petroleum origin. The compositions set forth in the tabulation were, in each instance, prepared by blending a concentrate with the lubricating base, the concentrate employed having the following composition:

| Concentrate:                    | Percent by weight |
|---------------------------------|-------------------|
| "Soap solution"                 | 64.6              |
| Tall oil                        | 5.2               |
| NaOH (50 Bé)                    | 3.0               |
| Diethylene glycol               | 5.5               |
| Ethylene glycol monobutyl ether | 12.7              |
| Water                           | 9.0               |
|                                 | 100.0             |

The ingredient shown as soap solution as used herein comprises about 60 percent of the water soluble sodium salts of mahogany acids derived from petroleum, about 5 percent water, and the balance mineral oil. The ingredients are shown in formula amounts, soaps being formed by action of the sodium hydroxide with the tall oil prior to blending with the remaining constituents.

The extract employed in preparation of the extract-containing compositions in the tabulation was a furfural extract per se obtained from a Pennsylvania crude oil by subjecting the oil to distillation from which a pressable distillate was obtained, said distillate being press dewaxed and subjected to distillation to remove gas oil and yield a bottoms fraction. The bottoms fraction was then solvent extracted with furfural to yield an extract, comprised predominantly of aromatic-containing molecules, having the following characteristics:

|                      |          |
|----------------------|----------|
| Gravity, API         | 7.8      |
| Flash point          | ° F. 405 |
| Fire point           | ° F. 475 |
| Viscosity at 100° F. | SUS 2765 |
| Viscosity at 210° F. | SUS 71.7 |
| Carbon residue       | 0.91     |

With reference to the compositions set forth in the tabulation, composition No. 1 relates to a conventional soluble oil in which the lubricating base is a mineral oil having a viscosity of 100 SUS at 100° F. and hence illustrative of mineral oils widely used in soluble oils. As shown, the soluble oil consisting of such a mineral oil and 19.2 percent of the concentrate as afore-described had a maximum water tolerance of about 4 percent. Such a soluble oil, containing water in such an amount, was a stable homogeneous oil composition that formed a stable emulsion when added to a relatively large proportionate amount of water. However, a soluble oil containing the same ratio of concentrate to mineral oil, but in which the amount of water was in excess of that shown as tolerated for composition 1, was cloudy in appearance. With further reference to the tabulation, compositions Nos. 2 to 4, inclusive show that, by use as a lubricating base of a mixture of the same 100 pale oil with the extract, liquid compositions were prepared that tolerated more water than composition 1. Such an increased water tolerance was obtained even though the same ratio of lubricating base to concentrate was used in compositions Nos. 2 to 4 as was used in composition 1. As is further shown, the compositions containing the extract possessed a higher water tolerance though the amount of soap present was less than that employed in composition 1, the lesser amount of soap being due to the presence of less concentrate in compositions 2 to 4 as compared to composition 1. Composition 5 relates to a soluble oil in which the lubricating base was the extract per se and, as shown, the water tolerance therefor was the same as composition 4 which differed from composition 5 in that the former contained a lubricating base composed of equal parts by weight of the extract and mineral oil. Upon further consideration of the data shown for composition Nos. 2 to 5 as compared to composition 1, it is evident that use of the extract as the lubricating base not only results in compositions having a higher water tolerance than those devoid of the solvent extract, but, of additional importance, show that, by use of a lubricating base composed of the extract in combination with a mineral oil, compositions of higher water tolerance may be obtained and in which the proportion of extract to mineral oil may be varied over a wide range to obtain higher water tolerances while at the same time enabling provision of soluble oils having desired viscosity characteristics that results by blending of the high viscosity extract with the lighter viscosity mineral oil.

Composition Nos. 6 to 8, inclusive, are similar to each other in the ratio of lubricating base to concentrate employed but contain mineral oil fractions of different viscosity characteristics in combination with the extract as the lubricating base. As shown, compositions 6 and 7 which contain the lighter viscosity pale oils, had the same water tolerance, whereas composition No. 8, which contained #2 fuel oil, showed a markedly increased water tolerance. The markedly increased amount of water tolerated by a composition such as No. 8 relates to a preferred

| Composition Number | Composition—Percent By Weight |                               |                              |                |               | Ratio of Lubricating Base to Concentrate in Soluble Oil |
|--------------------|-------------------------------|-------------------------------|------------------------------|----------------|---------------|---------------------------------------------------------|
|                    | Extract                       | Pale Oil (100 SUS at 100° F.) | Pale Oil (55 SUS at 100° F.) | No. 2 Fuel Oil | Concen- trate |                                                         |
| 1                  | 9.5                           | 76.8                          |                              |                | 19.2          | 4                                                       |
| 2                  | 9.5                           | 66.5                          |                              |                | 19.0          | 4:1                                                     |
| 3                  | 23.25                         | 51.15                         |                              |                | 18.6          | 4:1                                                     |
| 4                  | 36.4                          | 36.4                          |                              |                | 18.2          | 4:1                                                     |
| 5                  | 72.8                          |                               |                              |                | 18.2          | 4:1                                                     |
| 6                  | 57.85                         | 13.35                         |                              |                | 17.8          | 11                                                      |
| 7                  | 57.85                         |                               | 13.35                        |                | 17.8          | 11                                                      |
| 8                  | 53.95                         |                               |                              | 12.45          | 16.6          | 17                                                      |

aspect of the invention, i. e. the use in the compositions of a lubricating base that is a mixture of the extract with a low viscosity mineral oil fraction, the water tolerance thereof being greatly in excess of oil or extract alone as a lubricating base. Soluble oils as embodied herein are further characterized by possessing, when emulsified with a relatively large proportionate amount of water or in preparation for use, a relatively high load carrying capacity. In illustration thereof, the following tabulation sets forth several compositions as embodied herein in comparison with compositions similar thereto except that the lubricating base was a mineral oil and devoid of a solvent extract. The superiority of the compositions embodied herein as to load carrying effectiveness is shown by the data obtained on a Falex tester and in which test the loads were applied gradually while rotating the pin at a constant speed. This device, which is a well-known lubricant testing machine, comprises a steel pin rotatable between two non-rotatable steel jaws carrying V-shaped bearing surfaces and means for clamping the rotating pin between the bearing surfaces with adjustable force. In conducting the test, the oil emulsion under observation was kept in contact with the revolving pin while the latter was clamped between the bearings with steadily increasing force applied to the jaws. The amount of force, as indicated on the load guage of the machine, required to cause seizure between pin and bearings represents failure of the test composition.

extract to about one-fourth to about seven parts by weight of the mineral oil. Such relative proportions of the lubricating base are illustrated by the ratio of one part of extract to about seven parts of oil in composition 2 of the aforesaid tabulation, and to about one-fourth part of oil as in composition Nos. 6 to 8.

Moreover, and due to the exceptionally wide range of water tolerated by compositions as embodied herein, it is obvious that such compositions may be prepared that contain water in amounts that vary considerably based on the weight of the compositions. In broad aspect, therefore, the amount of water present in the composition should be sufficient to inhibit gelation but less than an amount sufficient to induce ingredient separation. Although the amount of water tolerated by compositions as embodied herein depends on factors such as the amount of extract in the lubricating base, or the amount of mineral oil used therewith, or the amount of soap employed, or the like, it is apparent from the foregoing data that compositions containing as high as 20% water, and even higher, may be prepared that are stable homogeneous solutions and form stable oil-in-water emulsions, e. g. the type of emulsion desired in the use of soluble oils for preparation of lubricating and coolant compositions in metal fabricating operations. Illustrative of such compositions is No. 8 of the aforesaid tabulation which contains about 19% water consisting of the water present in the concentrate plus the

| Composition Number | Composition (by Weight) |         |                                             |             | Ratio of Lubricating Base to Concentrate | Emulsion of 10% of Composition and 90% Water |
|--------------------|-------------------------|---------|---------------------------------------------|-------------|------------------------------------------|----------------------------------------------|
|                    | Mineral Oil             | Extract | Water (Over and above water in concentrate) | Concentrate |                                          |                                              |
| 9                  | 80 (100 Pale)           |         |                                             |             | 20.0                                     | 4:1 1,000                                    |
| 10                 | 76.8 (100 Pale)         |         | 4.0                                         |             | 19.2                                     | 4:1 1,000                                    |
| 11                 | 77 (100 Pale)           |         |                                             |             | 23                                       | 3.3:1 1,000                                  |
| 12                 |                         | 80.0    |                                             |             | 20.0                                     | 4:1 3,500                                    |
| 13                 |                         | 72.8    | 9.0                                         |             | 18.2                                     | 4:1 3,500                                    |
| 14                 |                         | 77      |                                             |             | 23                                       | 3.3:1 3,500                                  |
| 15                 | 12 (#2 Fuel)            | 56      | 15                                          |             | 17                                       | 4:1 3,500                                    |

As aforescribed, the compositions of the present invention comprise a lubricating base, an emulsifying agent and water with the lubricating base generally being the major component based upon the weight of the composition. When, as aforescribed, the lubricating base comprises a mixture of the extract with a mineral oil, the relative proportion of extract to mineral oil in the lubricating base may be varied over a rather wide range depending upon factors such as the ultimate viscosity desired, obtainment of which is facilitated by blending of the viscous extract with a low viscosity mineral oil, the desired increase in water tolerance as compared to use of the mineral oil per se as the lubricating base, and the like. As to the mineral oil component of the lubricating base, suitable therefor are liquid fractions obtained as petroleum distillates, such as those having a viscosity up to about 200 SUS at 100° F., and in some instances even higher, but usage of low viscosity petroleum distillates such as those in the #2 fuel oil range (e. g. 35-40 SUS at 100° F., low viscosity pale oils (e. g. 55 SUS at 100° F.) and higher viscosity pale oils (e. g. 100 SUS at 100° F.), is preferred. Although the relative amount of a mineral oil fraction to extract may be varied, depending on factors such as aforesaid and, additionally, upon volatility characteristics desired for the soluble oil composition, highly suitable compositions as embodied herein comprise, as the major amount by weight based on the composition, a lubricating base that is a mixture of one part by weight of the

amount (17%) shown as water tolerated over and above that in the concentrate.

Although the present invention has been described in conjunction with certain preferred embodiments thereof, those skilled in the art will readily recognize that variations and modifications can be made. Such modifications and variations are to be considered to be within the purview of the specification and scope of the appended claims.

I claim:

1. A stable soluble oil composition comprising, in homogeneous solution, a lubricating base in major amount based upon the weight of said composition, a water soluble soap as an emulsifying agent, a coupling agent in an amount sufficient to disperse said soap in said lubricating base, and water in an amount sufficient to inhibit gelation but less than an amount sufficient to induce separation of said composition, said lubricating base comprising (a) a predominantly aromatic extract obtained by furfural extraction of a petroleum fraction and (b) a mineral oil fraction which has not been solvent extracted.

2. A composition, as defined in claim 1, wherein the mineral oil component of the lubricating base is a petroleum distillate.

3. A composition, as defined in claim 1, wherein the lubricating base contains the furfural extract in a weight ratio of one part of extract to about one-fourth to about seven parts of mineral oil.

4. A composition, as defined in claim 1, wherein the soap is a metal soap of an organic acid.

5. A stable soluble oil composition comprising, in homogeneous solution, a lubricating base in major amount based on the weight of the composition, a water soluble metal soap as an emulsifying agent, a coupling agent in an amount sufficient to disperse said soap in said lubricating base, and water in an amount sufficient to inhibit said composition against gelation but less than an amount sufficient to induce separation of said composition, said lubricating base being a blend of (a) a mineral oil fraction which has not been solvent extracted and (b) a predominantly aromatic extract obtained by furfural extraction of a petroleum bottoms fraction in an amount sufficient to impart to said composition a substantially increased water tolerance as compared to use of said mineral oil fraction per se as the lubricating base.

6. A composition, as defined in claim 5, wherein the mineral oil component of the lubricating base is a low viscosity mineral oil fraction and the soap is a water soluble metal soap of an organic acid.

7. A composition, as defined in claim 6, wherein the soap is a mixture of alkali metal salts of a mixture of mahogany acids and tall oil.

8. A composition, as defined in claim 5, wherein the coupling agent is a mixture of an alcohol and an alcohol ether.

9. A composition, as defined in claim 8, wherein the alcohol is diethylene glycol and the alcohol-ether is ethylene glycol monobutyl ether.

10. A stable non-emulsified soluble oil composition of improved water tolerance characteristics comprising, in homogeneous solution, as a lubricating base, in major amount by weight of said composition, a predominantly aromatic extract obtained by furfural extraction of a

5 mineral oil, a water-soluble soap as an emulsifying agent, a coupling agent in an amount sufficient to disperse said soap in said lubricating base, and water in an amount sufficient to inhibit said composition against gelation but

10 less than an amount sufficient to induce separation of said composition.

11. A stable non-emulsified soluble oil composition comprising, in homogeneous solution, a lubricating base in major amount based on the weight of the composition,

15 a water soluble soap comprising a mixture of alkali metal salts of petroleum mahogany acids and tall oil, a coupling agent comprising diethylene glycol and ethylene glycol monobutyl ether in an amount sufficient to disperse said soap in said lubricating base, and water in an amount

20 sufficient to inhibit said composition against gelation but less than an amount sufficient to induce separation of said composition, said lubricating base comprising (a) a mineral oil fraction which has not been solvent extracted from the group consisting of relatively low viscosity

25 pale oils and petroleum distillates of the #2 fuel oil viscosity range and (b) a predominantly aromatic extract obtained by furfural extraction of a petroleum fraction other than said mineral oil fraction, said extract being present in said lubricating base in an amount

30 sufficient to impart to said composition a substantially increased tolerance for water as compared to use of the mineral oil fraction per se as the lubricating base.

References Cited in the file of this patent

UNITED STATES PATENTS

|    |           |                      |               |
|----|-----------|----------------------|---------------|
| 30 | 2,304,125 | Shutt et al. _____   | Dec. 8, 1942  |
|    | 2,320,263 | Carlson et al. _____ | May 25, 1943  |
|    | 2,340,035 | Zimmer et al. _____  | Jan. 25, 1944 |
|    | 2,413,353 | Hunter et al. _____  | Dec. 31, 1946 |